

## UNITED STATES PATENT OFFICE

HORACE CAMPBELL HALL, OF LITTLEOVER, DERBY, AND TENNYSON FRASER BRADBURY, OF DERBY, ENGLAND, ASSIGNORS TO ROLLS ROYCE LIMITED, OF DERBY, ENGLAND

## ALUMINUM ALLOY

No Drawing. Application filed September 30, 1930, Serial No. 485,548, and in Great Britain October 1, 1929.

This invention is a modification of the invention described in application for Letters Patent Serial No. 401,970, now Letters Patent No. 1,782,300, of November 30, 1930, and the 5 modification thereof described in our concurrent application Serial No. 485,547 of the date of this application. In the said application for Letters Patent we have described an alloy compounded of the elements in the relative quantities as follows:—

|                                | Per cent of<br>the whole |
|--------------------------------|--------------------------|
| Copper                         | 0.5 to 5.0               |
| Magnesium                      | 0.1 to 1.7               |
| Nickel                         | 0.2 to 1.5               |
| 15 Iron                        | 0.6 to 1.5               |
| Silicon exceeding              | 0.55 to 2.8              |
| Titanium                       | up to 0.3                |
| Manganese                      | up to 0.3                |
| 20 Aluminium                   | the remainder            |
| Only traces of other elements. |                          |

In our concurrent application of the date of this application Serial No. 485,547 we have described a modification of the said alloy in 25 which the magnesium content exceeds 0.03 per cent but does not exceed 0.10 per cent. Alloys falling within the said ranges are hereinafter called the said alloys.

Since the date of our said application we 30 have discovered that the castings of the said alloys are more free from scum and pin holes, particularly on the upper surface, if a small quantity of metallic sodium not exceeding 0.01 per cent of the alloy to be treated is 35 plunged into the alloy when in a molten condition, and preferably immediately before the latter is poured into the mould. This process has the effect of cleaning and de-oxidizing the alloy.

40 The preferred method of applying the sodium is as follows: We take a small quantity of metallic sodium (not exceeding the aforesaid limit) and in order to delay the oxidization of the sodium as long as possible wrap it 45 in a piece of sheet aluminium or aluminium foil, and so wrapped plunge it into the molten alloy, and hold it below the surface thereof until it is diffused. The bulk of the sodium so added is lost through burning at the moment of immersion, and through the fluxing

and deoxidizing effect on the alloy, and only traces of it are left in the castings. We are aware that it has previously been proposed to modify the structure of aluminium alloys by the addition thereto of metallic sodium, but 55 the proposals have been to add the sodium in quantities considerably larger than that which we use (namely not exceeding 0.01 per cent of the alloy to be treated) which is insufficient to affect the structure of the alloy but yet is sufficient to effect the advantages before described.

What we claim is:—

1. As a process in making a casting of the following metals, to wit:

|                                | Per cent of<br>the whole |
|--------------------------------|--------------------------|
| Copper                         | 0.5 to 5.0               |
| Magnesium                      | 0.1 to 1.7               |
| Nickel                         | 0.2 to 1.5               |
| Iron                           | 0.6 to 1.5               |
| Silicon exceeding              | 0.55 to 2.8              |
| Titanium                       | up to 0.3                |
| Manganese                      | up to 0.3                |
| 20 Aluminium                   | the remainder            |
| Only traces of other elements. |                          |

before pouring the molten alloy into the mould, plunging into it a small quantity of metallic sodium not exceeding 0.01 per cent of the alloy to be treated.

2. A process as claimed in claim 1 the metallic sodium being plunged into the molten alloy immediately prior to the latter being poured into the mould.

3. A process as claimed in claim 1 the metallic sodium being held under the surface of the molten alloy until diffused.

In testimony whereof we have hereunto affixed our signatures.

HORACE CAMPBELL HALL. 90  
TENNYSON FRASER BRADBURY.